

1

3,053,677

**PETROLEUM WAX FOR PAPER COATINGS**  
 George P. Touey, Kingsport, Tenn., assignor to Eastman Kodak Company, Rochester, N.Y., a corporation of New Jersey  
 No Drawing. Filed Nov. 12, 1959, Ser. No. 852,225  
 7 Claims. (Cl. 106—162)

This invention concerns an improved type of petroleum wax for use in wax coating compositions, more particularly petroleum wax modified with an aliphatic acid ester of a sugar.

Petroleum waxes are well known in the paper coating field used for making waxed paper of various types. Waxed papers of this type are cheap and highly efficient in producing water-proof paper containers such as milk cartons, paper cups and the like for various types of beverages. These waxed papers are also used for wrapping various food items to protect them from dirt, dehydration, moisture and the like.

Not only are wax coatings inexpensive but they have the desirable features of being free flowing liquids in the melted state, frequently melting under 100° C. permitting paper to be coated by simply dipping or passing the paper through a hot melt of the material.

Although petroleum wax coatings are used extensively to water-proof paper, they have several shortcomings which have not been previously resolved successfully. For instance, they have poor scuff-resistance and poor resistance to impact. This means that the coatings are often scraped off of the paper in normal usage or are easily shattered by a heavy blow. Another disadvantage is that the coatings, being extremely non-polar in character, often do not bond sufficiently to the paper to permit folding of the paper without having the wax coating flake off.

As a means of avoiding these disadvantages, it has been suggested that plasticizers be added to the wax formulations to reduce their tendency to flake and to make them adhere more firmly to paper. However, the common plasticizers are not compatible with petroleum wax. Usually the plasticizer is not sufficiently soluble in the wax or in the event that it is soluble, it gradually exudes to the surface of the coating producing a sticky or glossy film.

We have discovered a more compatible plasticizer for petroleum wax which not only is compatible with petroleum wax but also provides a better adherence to the paper surface and reduces flaking when the paper is bent or folded.

One object of this invention is to disclose a new type of additive for petroleum waxes designed for coating operations. Another object is to disclose a new type of additive which is highly soluble in the wax and which will not exude to form a glossy or tacky surface. A third object is to disclose a new type of wax formulation which will bond more firmly to the paper than the petroleum wax alone. A fourth object is to disclose a new and more compatible plasticizer for petroleum wax. These objects are accomplished by blending certain types of sugar esters with the wax before it is used as a paper coating. The esters are substantially completely esterified aliphatic acid esters of glycose, sucrose, sorbitol and the lower alkyl glycosides such as methyl alpha-D-glycoside and ethyl alpha-D-glucoside.

The amount of sugar ester required depends on the type of ester and the amount of plasticizing and enhanced bonding action of the wax desired. Thus for some paper surfaces only as little as 2% of the sugar acid additive is all that is required, whereas in other applications the concentration of the sugar additive may be as high as

2

25%. Normally, however, a concentration of 3-15 parts sugar ester to 97-85 parts of petroleum wax is sufficient. Higher concentration of sugar esters, although suitable for certain specialized operations usually tend to make a tacky wax coating. The preferred concentration for general use in paper coatings is 3-10 parts sugar ester and 97-90 parts petroleum wax.

The sugar esters which function as plasticizers and bonding agents for the petroleum waxes are the substantially completely esterified aliphatic acid esters (containing 3-8 carbon atoms in their acyl substituents) of glucose, sucrose, sorbitol, methyl  $\alpha$ -D-glucoside. Thus, the propionic, butyric, isobutyric, valeric, isovaleric, hexanoic, isohexanoic, heptanoic, octanoic, and 2-ethylhexanoic acid esters of these sugars may be employed. Also the aliphatic acids can be unsubstituted as in the case of crotonic, methacrylic, and the like.

Sugar esters with aliphatic acyl groups containing more than 8 carbon atoms such as, for example, sucrose octopalmitate or octaoleate are undesirable. These are not sufficiently compatible with the wax and gradually exude to the surface of the wax after standing several weeks. The aromatic acid esters are undesirable for similar reasons. In addition, aromatic acid esters of sugars in general are considered more toxic than the aliphatic acid esters.

The preferred sugar esters are the isobutyrate esters of glycose, sucrose, sorbitol and methyl (or ethyl) alpha-D'-glucoside. They can be made by inexpensive procedures, impart no objectionable odor to the wax, and they have a sufficient number (4) of carbon atoms on their acyl substituents to provide the proper amount of solubility in the wax. Also, they are completely water-insoluble and are quite stable to heat. The glucose and sucrose esters are readily made by heating the acid anhydride and the sugar in the presence of a trace of sodium of potassium acetate catalyst. The sorbitol and methyl (or ethyl) glucoside esters can be esterified with the aliphatic acid directly using conventional catalysts.

Although it is preferred that the sugar esters be completely esterified, traces of un-esterified hydroxyl groups may remain in the product. However, this amount should be an average of no more than 1 hydroxyl group per 1 sugar molecule since the presence of a substantial amount of unesterified hydroxyl groups in the product tends to make it less compatible with the wax.

The petroleum waxes of this invention are those hydrocarbon fractions which have a melting point range of from above about 40° C. to about 96° C. The main two waxes in this classification are the paraffin waxes (melting point 43-66° C.) and the microcrystalline waxes (melting point 63-94° C.). These are the petroleum waxes used by the paper coating industry. It is understood, however, that these waxes can contain a minor proportion of the various polyolefin waxes. The polyolefin waxes may be used in concentrations up to 1 part polyolefin wax to 9 parts petroleum wax without any effect on the compatibility of the sugar esters with the petroleum wax.

#### EXAMPLE 1

This example illustrates the compatibility of the sugar esters of this invention with a standard grade of paraffin wax (M.P. 55° C.).

Ten grams of the sugar ester (Table I) was mixed with 90 g. of the melted paraffin wax at a temperature of 100° C. When thoroughly mixed, the hot solution was rated for its clarity. A clear solution indicated that the sugar derivative had dissolved completely in the wax, whereas a hazy solution or a two-layer system denoted incompatibility.

After the compatibility test was performed, the melted wax was then poured into a shallow dish, whereupon it solidified. The solidified product was stored for one week at 78° F. and 55% relative humidity. Any exudation of the sugar ester was noted after this storage period.

Table I

| Sugar Ester                                          | Compatibility Rating at 100°C. | Observation of Exudation                        |
|------------------------------------------------------|--------------------------------|-------------------------------------------------|
| Glucose pentaacetate                                 | Insoluble                      | Crystals of sugar ester on surface.             |
| Glucose pentapropionate                              | Partly soluble                 | A trace of sugar ester crystals on the surface. |
| Glucose pentabutyrate                                | Soluble                        | No exudation.                                   |
| Glucose pentaisobutyrate                             | do                             | Do.                                             |
| Glucose pentavalerate                                | do                             | Do.                                             |
| Glucose pentadecanoate                               | do                             | Slightly greasy surface.                        |
| Glucose pentaoleate                                  | do                             | Greasy liquid on surface.                       |
| Sucrose octaacetate                                  | Insoluble                      | Crystals of sugar ester on surface.             |
| Sucrose octapropionate                               | Partly soluble                 | A trace of sugar ester crystals on surface.     |
| Sucrose octabutyrate                                 | Soluble                        | No exudation.                                   |
| Sucrose octaisobutyrate                              | do                             | Do.                                             |
| Sucrose octavalerate                                 | do                             | Do.                                             |
| Sucrose octa-2-ethyl-hexanoate                       | do                             | Do.                                             |
| Sucrose octadecanoate                                | do                             | Slightly greasy surface.                        |
| Sucrose octastearate                                 | Partly soluble                 | Greasy solid particles.                         |
| Sorbitol hexaacetate                                 | do                             | Crystals of sugar ester on surface.             |
| Sorbitol hexapropionate                              | do                             | A trace of sugar ester crystals on the surface. |
| Sorbitol hexabutyrate                                | Soluble                        | No exudation.                                   |
| Sorbitol hexaisobutyrate                             | do                             | Do.                                             |
| Sorbitol hexavalerate                                | do                             | Do.                                             |
| Sorbitol hexa-2-ethyl-hexanoate                      | do                             | Do.                                             |
| Sorbitol hexaoctadecanoate                           | do                             | Slightly greasy surface.                        |
| Sorbitol hexopalmitate                               | do                             | Greasy solid particles on surface.              |
| Methyl $\alpha$ -D-glucoside tetraacetate            | do                             | Crystals of sugar ester on surface.             |
| Methyl $\alpha$ -D-glucoside tetrapropionate         | do                             | No exudation.                                   |
| Methyl $\alpha$ -D-glucoside tetrabutyrate           | do                             | Do.                                             |
| Methyl $\alpha$ -D-glucoside tetraisobutyrate        | do                             | Do.                                             |
| Methyl $\alpha$ -D-glucoside tetravalerate           | do                             | Do.                                             |
| Methyl $\alpha$ -D-glucoside tetra-2-ethyl-hexanoate | do                             | Slightly greasy surface.                        |
| Methyl $\alpha$ -D-glucoside tetraoctadecanoate      | do                             | Do.                                             |
| Methyl $\alpha$ -D-glucoside tetrapalmitate          | do                             | Greasy surface.                                 |

The compatibility tests show that the sugar esters with acyl constituents containing more than 8 carbon atoms are compatible with the melted wax but gradually exude to the surface of the wax when it solidifies. This is probably because they are not sufficiently soluble in the wax at room temperature. The sugar acetates and some of the propionates were either insoluble in the melted wax or insoluble in it when it returned to room temperature. The tests also show that those esters with acyl carbon numbers between 3 and 8 were considerably more soluble in the wax and had little or no tendency to exude to the surface of the solidified wax.

**EXAMPLE 2**

This example illustrates how the wax coatings containing the wax-compatible sugar esters did not flake off when the coatings were bent.

An uncoated milk-carton grade of heavy paper was cut into strips of 2" x 6". A strip of this paper was submerged in each of the hot melts shown on Table II for 5 minutes. The temperature of the melts was maintained between 95° and 100° C. during this operation. After the strips were thoroughly wetted with the liquid wax, they were removed and allowed to come to room temperature. They were then stored for 24 hours at 78° F. and 55% relative humidity before they were tested.

The coated strips were bent to an angle of 180° and the degree of flaking of the wax along the crease was

observed. This operation was repeated until flaking of the wax in all cases was finally observed.

|    |                                                          | Number of<br>Folds Re-<br>quired to<br>Cause the<br>Wax to<br>Flake off<br>the Paper<br>at the Crease |
|----|----------------------------------------------------------|-------------------------------------------------------------------------------------------------------|
| 5  | Sugar Ester in the Wax Coating 1                         |                                                                                                       |
| 10 | Glucose pentapropionate.....                             | 6                                                                                                     |
|    | Glucose pentabutyrate.....                               | 8                                                                                                     |
|    | Glucose pentaisobutyrate.....                            | 7                                                                                                     |
|    | Glucose pentavalerate.....                               | 9                                                                                                     |
|    | Sucrose octapropionate.....                              | 7                                                                                                     |
|    | Sucrose octabutyrate.....                                | 12                                                                                                    |
|    | Sucrose octaisobutyrate.....                             | 14                                                                                                    |
| 15 | Sucrose octavalerate.....                                | 11                                                                                                    |
|    | Sucrose octa-2-ethylhexanoate.....                       | 13                                                                                                    |
|    | Sorbitol hexapropionate.....                             | 5                                                                                                     |
|    | Sorbitol hexabutyrate.....                               | 8                                                                                                     |
|    | Sorbitol hexaisobutyrate.....                            | 9                                                                                                     |
|    | Sorbitol hexavalerate.....                               | 9                                                                                                     |
|    | Sorbitol hexa-2-ethylhexanoate.....                      | 10                                                                                                    |
| 20 | Methyl $\alpha$ -D-glucoside tetrapropionate.....        | 7                                                                                                     |
|    | Methyl $\alpha$ -D-glucoside tetrabutyrate.....          | 8                                                                                                     |
|    | Methyl $\alpha$ -D-glucoside tetraisobutyrate.....       | 9                                                                                                     |
|    | Methyl $\alpha$ -D-glucoside tetravalerate.....          | 10                                                                                                    |
|    | Methyl $\alpha$ -D-glucoside tetra-2-ethylhexanoate..... | 10                                                                                                    |
|    | No sugar ester (control).....                            |                                                                                                       |

25 <sup>1</sup> Except for the control coating, all of the waxes consisted of 90 parts paraffin wax and 10 parts sugar ester.

This nonflaking characteristic of the wax is caused by a two-fold effect. The first is the more polar nature of the ester in comparison with the wax. This tends to give 80 a stronger bond to the paper. The other is the plasticizing action which the ester has on the wax.

The polyolefin waxes which can be admixed with the petroleum-sugar ester combinations of this invention are chosen from those polyethylene and polypropylene waxes which are compatible with the petroleum waxes. Their molecular weights range from about 1000 to 10,000 and their melting points are within the limits of 70° C. and 120° C.

120 C.

40 1. A wax coating composition consisting essentially of a petroleum wax consisting of those hydrocarbon fractions having a melting point range of from about 40° C. to about 96° C. and 0-10% of a polyolefin wax selected from the class consisting of polyethylene and polypropylene 45 waxes having a molecular weight range of 1,000 to 10,000 and melting points within the range of 70° C. and 120° C., and 2-25%, based on the total weight of the composition, of a sugar ester, having an average of no more than one hydroxyl group per sugar molecule, selected 50 from the class consisting of the esters of glucose, sucrose, sorbitol, and the lower alkyl glucosides obtained by reacting the sugar with an acid selected from the class consisting of propionic, butyric, isobutyric, valeric, isovaleric, hexanoic, isohexanoic, heptanoic, octanoic, 2-ethyl 55 hexanoic, crotonic, and methacrylic acids.

2. A coating composition consisting essentially of a petroleum wax consisting of those hydrocarbon fractions having a melting point of 40-96° C. and 2-25%, based on the weight of the coating composition of a substantially 60 completely esterified isobutyrate sugar ester obtained from glucose.

3. A coating composition consisting essentially of a petroleum wax consisting of those hydrocarbon fractions having a melting point of 40-96° C. and 2-25%, based 65 on the weight of the coating composition, of a substantially completely esterified isobutyrate sugar ester obtained from sucrose.

4. A coating composition consisting essentially of a petroleum wax consisting of those hydrocarbon fractions 70 having a melting point of 40-96° C. and 2-25%, based on the weight of the coating composition, of a substantially completely esterified isobutyrate sugar ester obtained from sorbitol.

5. A coating composition consisting essentially of a 75 petroleum wax consisting of those hydrocarbon fractions

having a melting point of 40-96° C. and 2-25%, based on the weight of the coating composition, of a substantially completely esterified isobutyrate sugar ester obtained from methyl- $\alpha$ -D'-glucoside.

6. A coating composition consisting essentially of a petroleum wax consisting of those hydrocarbon fractions having a melting point of 40-96° C. and 2-25%, based on the weight of the coating composition, of a substantially completely esterified isobutyrate sugar ester obtained from ethyl- $\alpha$ -D'-glucoside.

7. A waxed paper comprising a paper substrate having thereon a coating composition consisting essentially of a petroleum wax consisting of those hydrocarbon fractions having a melting point range of from about 40° C. to about 96° C. and 0-10% of a polyolefin wax selected from the class consisting of polyethylene and polypropylene waxes having a molecular weight range of 1,000 to 10,000 and melting points within the range of 70° C. and 120° C., and 2-25%, based on the total weight of the composition, of a sugar ester, having an average of no

10

15  
20

more than one hydroxyl group per sugar molecule, selected from the class consisting of the esters of glucose, sucrose, sorbitol, and the lower alkyl glucosides obtained by reacting the sugar with an acid selected from the class consisting of propionic, butyric, isobutyric, valeric, isovaleric, hexanoic, isohexanoic, heptanoic, octanoic, 2-ethyl hexanoic, crotonic, and methacrylic acids.

## References Cited in the file of this patent

## UNITED STATES PATENTS

|           |          |               |
|-----------|----------|---------------|
| 2,094,771 | Church   | Oct. 5, 1937  |
| 2,108,808 | Finzel   | Feb. 22, 1938 |
| 2,322,198 | Parsons  | June 15, 1943 |
| 2,700,022 | Clayton  | Jan. 18, 1955 |
| 2,733,225 | Smith    | Jan. 31, 1956 |
| 2,783,156 | Oathont  | Feb. 26, 1957 |
| 2,791,510 | Sproule  | May 7, 1957   |
| 2,893,990 | Haas     | July 7, 1959  |
| 2,908,681 | Anderson | Oct. 13, 1959 |